

## UNITED STATES PATENT OFFICE.

GEORGE FREEMAN LLOYD, OF BRIGHTON, VICTORIA, AUSTRALIA, ASSIGNOR TO SPEC-  
TRUM DYES PROPRIETARY LIMITED, OF MELBOURNE, S. C. 4, AUSTRALIA, A COM-  
PANY OF VICTORIA.

## DYING OF FABRIC.

No Drawing. Application filed April 6, 1928, Serial No. 268,076, and in Australia February 6, 1928.

This invention relates to the treatment of dyed fabrics and its object is to enable the colour of a dyed fabric to be transformed to a lighter colour. The word colour is 5 used herein in its wide sense to include a shade of colour.

In the past it has been known to strip dark colours from fabrics and, after this complete removal of the colours dyed 10 thereon, to redye the fabrics to the particular colour desired.

I have found that, instead of completely stripping the colour from the fabric, it is possible to produce selectively any one of a 15 range of intermediate lighter colours by a controlled semi-stripping process in which the reduction of the colour is regulated by the control of the temperature as well as by selection of the proportions of the reagents.

20 These temperatures and proportions are predetermined by test for each material to produce the particular colour selected out of the range available. Colours not in the available range may be obtained by transforming the darker colour to a lighter colour approximating that desired and then obtaining 25 the exact colour by a slight amount of dyeing.

The stripping agents employed in this 30 process and the proportions in which they are used are selected so that the action proceeds slowly. This facilitates the controlling of the process so that by exact selection of the concentrations of the reagents and of 35 the temperatures a uniform end point can be predetermined for the production of the desired colour with an exceedingly level finish.

As the dyes which are to be converted and 40 the materials to be treated vary considerably in their nature, the reagents used and their proportions must be varied. Thus, to treat aniline dyes on fabrics formed of cotton, cotton unions (with wool or silk), or silk, the 45 material is treated in a wooden vat which contains a sheet of perforated zinc, the material being kept out of actual contact with the zinc by a perforated false bottom. Cold water is placed in the vat, before the material 50 is inserted, in sufficient quantity to cover the material and 1% (one per cent) of sodium bisulphite ( $\text{NaHSO}_3$ ) is then added. The material is thoroughly saturated with the solution and is next lifted out of the 55 solution either by rolling it up on a winch

or otherwise. A second solution is prepared by adding 1 lb. of pure zinc dust to 1 gallon of commercial solution of sodium bisulphite. In place of the sodium bisulphite a mixture of sodium sulphite and sodium sulphate may 60 be used, just as is well known in the case of ordinary stripping treatment. In either case the mixture is allowed to stand for about half an hour and is then decanted off without disturbing the sediment. 2% (two 65 per cent) of coal tar naphtha is next added to either the first or the second solution, the function of the coal tar naphtha being to promote the penetration of the treated fabric by the reagent, and the brightening of the 70 shade of the dye under conversion. This second solution is then added to the first solution in the vat in the proportion of about 1 gallon of second solution to every 25 gallons of first solution contained in the vat. 75

The temperature is then raised to approximately 60° C. and the fabric is then returned to the vat and kept in motion. The liquor in the vat is then raised gradually to the particular temperature which has been determined beforehand, by testing, to correspond to the particular colour desired. In this testing a small piece of the material is treated by equivalent processes in the laboratory under conditions estimated to be correct, 85 and, if the desired colour is not produced, the conditions are modified to the necessary extent as determined by further trial and the whole fabric is then treated under the conditions thus determined. The stopping 90 of the process sharply at the desired end point with a level colour is facilitated in a remarkable degree by the addition of about 2% (two percent) of 30% (thirty per cent) acetic acid or 5% (five per cent) of commercial solution of sodium bisulphite. This 95 step is a safeguard which enables the action to be stopped at the correct end point even if the control of the process is otherwise carelessly effected. The material is then 100 washed out thoroughly in a 5% (five per cent) solution of sodium bisulphite which fixes the dye.

To treat aniline dyes on woollen fabrics the material is first heated up in a bath containing 5% (five per cent) of coal tar naphtha. It is then removed from this bath and treated in the same way as above-described in connection with the treatment of dyed cotton, silk or unions.

I claim:

1. A process of lightening the colour of a dyed fabric down to any preselected point on the available range of colour consisting in subjecting the fabric to a uniformly and selectively controlled semi-stripping process with water containing the products of the reaction of sodium bisulphite with zinc, with the addition of coal tar naphtha.
- 5 2. A process of lightening the colour of a

dyed fabric down to any preselected point on the available range of colour consisting in subjecting the fabric to an incomplete stripping process, controlling the stripping process by regulating the concentration and 15 temperature of the stripping liquor, and finally fixing the resultant colour by addition of a fixing reagent.

In testimony whereof I affix my signature.

GEORGE FREEMAN LLOYD.